

Dec. 4, 1934.

W. J. POLYDOROFF

1,982,689

MAGNETIC CORE MATERIAL

Filed March 16, 1931

2 Sheets-Sheet 1

Fig. 1.



Fig. 2.



Fig. 3.



Fig. 4.



Fig. 5.



Fig. 6.



Fig. 7.



Fig. 8.



Fig. 9.



Fig. 10. Fig. 11.



Inventor:  
Vladimir J. Polydoroff,  
by Thomas G. Stevens

Dec. 4, 1934.

W. J. POLYDOROFF

**1,982,689**

### MAGNETIC CORE MATERIAL

Filed March 16, 1931

2 Sheets-Sheet 2



## UNITED STATES PATENT OFFICE

1,982,689

## MAGNETIC CORE MATERIAL

Vladimir J. Polydoroff, Chicago, Ill., assignor to  
 Johnson Laboratories, Incorporated, Chicago,  
 Ill., a corporation of Illinois

Application March 16, 1931, Serial No. 523,112

79 Claims. (Cl. 175—21)

The invention relates to magnetic cores used with inductance coils and transformers employed in high-frequency circuits, and said invention involves a new magnetic core material, a new magnetic core, and various new methods of producing said core material and said core.

Hitherto, several methods of producing a core material suitable for frequencies of the order of 10,000 cycles per second were known. In practicing these old methods, various finely-divided alloys with attempted insulation of each grain from the others were employed, the main object being to impart to the cores of loading coils, and other similar inductances used in telephone work at moderately low frequencies, a high initial permeability (permeability at low magnetizing intensity).

As core losses rapidly increase with frequency, cores of the old type become inoperative at frequencies of the higher orders, such as 150 to 1500 k. c., to which range the present invention more particularly relates. Requirements for core permeability are considerably smaller for high frequencies than for the low frequencies employed in telephone work, and the present invention has for an object the production of magnetic core materials and cores that are suitable for use at these high frequencies. Such cores may be conveniently described as comminuted to indicate that the magnetic material is finely divided.

The invention will be better understood if reference be made to the accompanying drawings, in which—

Figure 1 shows particles of magnetic material used in cores made in accordance with the present invention, as they appear when highly magnified;

Figures 2 and 3 show the same material in two stages of its preparation, in imaginary cross-section;

Figures 4, 5, 6, 7, 8, 9, 10 and 11 represent various shapes of magnetic cores made of the new finely divided material; and

Figures 12 and 13 diagrammatically indicate magnetic and electrical characteristics of cores embodying the invention.

It was shown by Currie, U. S. Patent No. 421,067 of 1890, that, for high-frequency work, magnetic cores should be made of small insulated iron particles and pressed into a suitable shape. Investigation of iron powders disposed in the field of a coil operating at frequencies of the order of 1000 kilocycles shows that the inductance increase due to the iron is of the order of 3 to 4 times, and, if the particles are of very small dimensions, the total losses occurring in the coil

will be small enough to permit successful operation in a radio circuit.

In the electrical arts, the term "apparent permeability" is usually taken as the ratio of the inductance as increased by the iron, to the air-core inductance, the measurement being made with a core of a substantially closed type, designed to enclose practically all the lines of force of the coil. In this specification and in the claims, I have used the term "apparent permeability" in this sense, but I use the term "effective permeability" to indicate this same inductance ratio, without regard to whether the core totally or only partially surrounds and encloses the field of the coil.

When a core is intended to be used for inductance variations over a wide range of frequencies, such as is employed in broadcasting, the effective permeability must be of the order of 8. It is plainly evident, therefore, that loose powdered iron cannot be used to fulfill the requirements of a radio circuit, and that, in order to increase the permeability, the loose powdered iron should be compressed into a more compact form. In this way, the particles may be so closely related as to produce the desired effective permeability.

At high frequencies, such as mentioned, the core losses are very pronounced and may be classified as: 1. Hysteresis losses, and 2. Eddy current losses. Hysteresis losses mainly depend upon the atomic structure of the magnetic material, and are small for materials of low magnetic coercivity, such as pure iron, Swedish iron, etc. Eddy current losses depend upon the surface areas of the magnetic particles, the minute induced currents circulating in the surface layers. The smaller the particles, the smaller the losses, and from this it is evident that, if several particles are in electric contact and the paths are thus increased in length, the resultant losses are also increased. Therefore, insulation of the individual magnetic particles is required, when these particles are pressed into compact masses. Eddy current losses also depend on the specific resistance of the magnetic material, an increase of which reduces the minute currents. Very often, however, an increase of resistivity, produced by alloying the metals, increases coercivity and therefore also increases hysteresis losses.

Different magnetic powders, including various alloys producing high initial permeability, were tried, the necessary particle size being produced by mechanical, electrolytic, or chemical processes. A preferable chemical process would be the reduction of a suitable iron compound by hy-

drogen. It was found that, although pure iron has a comparatively low initial permeability, the hysteresis losses in such iron are considerably less than in magnetic alloys.

5 A study of iron powder, reduced by hydrogen, indicates that the reduction can best be made from pure oxides  $Fe_2O_3$ ,  $Fe_3O_4$ , because these materials occur in a finely divided state. Reduced at high temperatures in a stream of hydrogen, 10 the oxides are converted into pure metallic iron particles of crystalline form, having plainly visible sharp edges, as seen under the microscope, the size of the crystals being of the order of .001 millimeter. The apparent specific density of 15 such reduced iron, when packed in a test tube, should be between 2.4 and 3.7.

As is shown in Figure 1, these crystals may group together to form masses of the order of .005 millimeter, these being sponge-like bodies 20 falling freely through a screen having 400 meshes to the inch, a variation of the temperature and the speed of reduction producing smaller or larger particles.

Although particles smaller than those above 25 described can easily be obtained by the aforesaid method, it is preferable, because of their ability to be more readily compressed into compact cores, to use particles of substantially the described dimensions, for the frequency range above mentioned.

The iron powder thus obtained is then thoroughly insulated so that each individual particle is coated with a thin film of a solid, but not brittle, insulating substance. The particles will 35 then be substantially insulated from one another when they are later molded into a compressed core. Various insulating methods were tried in an effort to discover an electrical insulation that would offer adequate mechanical resistance to 40 pressure, and insulations having this characteristic were finally developed.

In one method, iron powder of dimensions substantially as above described is mixed with a solution of phenol resin in acetone or other suitable 45 solvent, said solution being made thoroughly fluent. The amount of phenol resin in relation to the iron should be approximately 4 to 10 per cent. of the weight of the iron. The ingredients of this mixture are thoroughly blended, and the 50 product is then dried in air, and then baked in an oven, the insulating material being thus chemically converted into a stable compound. Care should be taken to prevent the formation of 55 cakes or lumps, so that the particles will remain substantially loose, and each particle will be individually coated and baked. This may be accomplished by suitable agitation.

Another method of insulating the particles is to use a varnish capable of being oxidized, such as 60 four parts of China-wood oil and one part of resin. Varnish of this composition may be thinned out by a suitable solvent such as toluol or benzine to the required fluency and then mixed with the iron powder, the varnish being from 65 2% to 5% of the weight of the iron after the volatile matter has evaporated.

The advantage of such a varnish is that its surface is oxidized very quickly, and this prevents 70 caking or lumping of the particles. The mixture is then put in an oven and thoroughly baked at an elevated temperature for several hours, thus integrating the insulating substance until a hard, yet elastic coating is obtained on the particles.

75 It is essential of course, to maintain the mate-

rial in the powdered form. The powder thus prepared should be appropriately tested in order to determine that the coatings on the particles are chemically stable, heat resistant and insoluble.

It will be understood that the materials above described for the individual insulation of the particles are of organic nature but that equivalent inorganic or synthetic substances may, of course, be substituted.

The insulated crystalline particles thus produced (Figure 2), are now to be bound together into a single coherent mass (Figure 3). Various binding substances, such as phenol resin, natural resin, and synthetic gums, either in liquid or dry powdered form, may be employed, and should be thoroughly mixed with the insulated iron powder. If a binder in solution is used to secure the mixture, the solvent must then be thoroughly dried out. The amount of binder may vary, but in the resulting cores it should not exceed 10% of the weight of the iron. If the insulating substance is a China-wood oil varnish, in quantity 3% of the weight of the iron, the amount of phenol resin used as a binder 100 should be approximately 7%, so that the compressed core will contain not more than 10% of inert materials against 90% of magnetic material by weight.

Cores of any desired shape may be made from 105 these materials, in molds heated to a temperature of about 100° C. While in the molds, the mixture is subjected to a pressure of from 5 to 25 tons per square inch, depending upon the shape of the core. This application of pressure 110 reduces the core to approximately four-tenths of its initial volume, the particles being thus so closely related as to produce useful values of effective permeability in the resulting cores. Figures 4, 5, 6, 7, 8, 9 and 11 indicate various shapes 115 of cores made in this way, and for use, respectively, with solenoidal coils (Figures 4 and 10), toroidal coils (Figure 5), binocular or figure-eight coils (Figure 6) and solenoids with substantially closed magnetic fields (Figures 7, 8, 120 9 and 11). The cores for use with solenoidal and binocular coils are all shown as being of circular cross-section but cores of any desired form may be molded.

When a heated core is thus compressed, a considerable displacement of particles occurs, and the pressure to which it is subjected may break the insulating films and establish longer paths for eddy currents. It is, therefore, preferable that, in order to preserve the insulation of the individual particles, the insulating films should be elastic and the binding substance somewhat plastic, during compression. The plasticity of the binding substance affects the magnetic and electrical properties of the cores, and, therefore, 135 it should be carefully controlled to produce the desired results.

One method of controlling the plasticity of the binder is to mix the insulated iron powder with dry powdered phenol resin, to heat the mixture to a temperature of 100 degrees centigrade, the mold being heated to the same temperature, and to then press the core while in said mold.

Another method is to mix the insulated iron powder with the phenol resin varnish, and to 145 then press it after the major part of the solvent of said varnish has been evaporated, and while the mixture is slightly tacky.

Still another method is to add to the dry mixture of iron powder and phenol resin powder, a 150

minute amount of solvent so as to make the binder semi-plastic.

Still another method is to mix the iron powder with natural resin in powdered form, and to 5 heat the mixture until said resin becomes plastic.

Liquid binders should be avoided because, under pressure in the mold, they tend to flow away from the iron, leaving some of the particles unbound.

10 The preferable treatment after passing depends on the nature of the binder. In the case of certain resins, the cores may be merely allowed to cool. If condensation products are used, the cores may be baked in an oven or in 15 a mold at an elevated temperature, until the binding material is converted by polymerization into a chemically stable product.

Of the above described methods of insulation, binding and compression, I prefer the use of the 20 China-wood oil resin varnish for insulation, and dry bakelite powder or bakelite varnish as a binder. The plasticity of the binder is efficiently controlled by heating the mixture to a definite temperature and pressing it in heated molds. I 25 also prefer to take the compressed product out of the mold for subsequent baking, although baking in the mold may be satisfactory in some cases. In either case the binder should be converted into a chemically-stable bakelite.

30 One advantage of releasing the pressure, and then heat treating the still incomplete compressed core, as for instance in an oven, as a finishing operation, is that, when the binder is in a plastic or softened state, the insulated magnetic particles have an opportunity to become 35 somewhat released and have a tendency to acquire an increased separation, which is indicated by the fact that the finished core is slightly expanded, the result being a material decrease of the eddy current losses. This is particularly true where a very elastic insulating medium, such as a China-wood oil varnish, is employed.

40 Cores produced by the methods above described have satisfactory mechanical strength, are capable of being mechanically worked like metals, and have the following characteristics:

Specific density, 4 to 5

45 Specific resistance, 10 to 50 ohms per centimeter cube.

The apparent permeability of a core of ring shape such as that shown in Figure 5 will be 50 of the order of 8. A core of the type shown in Figure 4, fitted to a solenoidal coil having a length of 50 millimeters and a diameter of 25 millimeters, will have an effective permeability 55 of from 4 to 5. A core similar to that shown in Figure 6, for a binocular coil composed of two solenoids of the same dimensions, will have an 60 effective permeability of about 6. The cores of Figures 7, 8, 9 and 11 which are arranged to almost completely surround a solenoidal coil, have effective permeabilities of approximately 8.

65 These values are for a frequency of 500 kilocycles per second, and a magnetic intensity of .1 gauss, but the apparent permeability remains substantially constant for a wide band of frequencies between 1 k. c. and 500 k. c., and a wide range of magnetizing forces between .01 and 10 gauss.

70 Figures 12 and 13 diagrammatically show the electric and magnetic characteristics of two different shapes of core.

75 The losses due to the core at high frequency may be conventionally expressed in ergs per cubic

centimeter per cycle at unit induction. Curve a of Figure 12 shows the core losses of the usual toroidal core between 50 and 450 k. c. The shape of the curve indicates that losses increase with frequency. The curve b, being a horizontal straight line, indicates that the permeability remains substantially constant. The core loss at 200 k. c., as indicated by the curve, is about .008 erg per cubic centimeter per cycle.

80 It is usual in high-frequency work to express the losses in terms of the effective radio-frequency resistance of a coil, and the same principle may be applied to an iron core used in conjunction with an inductance. The diagram shown in Figure 13 plots factors thus derived, the measurements being made at frequencies between 300 and 1400 k. c., on a specimen core of suitable shape. The curve c represents radio-frequency resistance in ohms for an iron core of the shell type. The permeability is shown by the graph d which is a straight line. The solenoidal coil used in making these measurements was placed in the annular cavity in the core, so that the core substantially enveloped the field of the coil.

85 The inductance L of the coil and its radio-frequency resistance R may be measured at any chosen frequency and the ratio

$$\frac{L}{R}$$

90 calculated. The core may then be inserted in the coil. The increase of effective inductance  $\Delta L$  and the increase of resistance  $\Delta R$  due to the iron may then be measured, and the term

$$\frac{\Delta L}{\Delta R}$$

95 computed. It will be found that for the same core material the term

$$\frac{\Delta L}{\Delta R}$$

100 varies considerably with different shapes of core, such as shown in Figures 4, 5, 6 and 7, but that for a given shape it remains substantially constant, regardless of the inductance and resistance 105 of the coil by itself. The ratio

$$\frac{\Delta L}{\Delta R}$$

110 may be conveniently taken as the factor of merit 115 of the core, because this ratio completely indicates the effect which the core will have upon any suitable inductance with which it is associated.

115 For differently shaped cores,

$$\frac{\Delta L}{\Delta R}$$

120 is different, but for the same core with different coils, it remains substantially constant and is of 125 the order of  $3 \times 10^{-6}$  for toroidal coils,  $25 \times 10^{-6}$  for solenoidal coils and  $10 \times 10^{-6}$  for a solenoid with closed magnetic field, L being stated in henrys and R in ohms.

130 Cores such as those shown in Figures 4, 5, 6 and 7 may be stationary or they may be arranged to be movable relatively to the coil. In the latter case, movement of the core produces a gradual change of the effective inductance of the coil, and thus may be utilized to tune a resonant circuit to various frequencies. Inductance is at a minimum when the core is withdrawn, corresponding to the highest frequency of the tuning range. As the core is gradually inserted into the coil, the effective inductance gradually increases, 145 150

until, when the core is all the way in, the maximum value of effective inductance is obtained, corresponding to the lowest frequency of the tuning range.

It has been found that with a movable type core the ratio

$$\frac{L+\Delta L}{R+\Delta R}$$

varies over the tuning range, as shown by curve *c* of Figure 13.

In radio-frequency reception it may be advantageous to maintain this ratio constant throughout the range of frequencies. The losses introduced by the initial portions of a homogeneous core at the higher frequencies may be considerably higher than would be permissible, but provision may be made for reducing the losses of the initial portion of the core, that is, the portion of the core which first enters the coil and which will be adjacent to the air gap, in the usual case. The reduction involves a slight sacrifice of permeability in this portion. It may be conveniently called "varying magnetic density" of the core. Curve *f* of Figure 13 shows that, with such a core, the factor

$$\frac{L+\Delta L}{R+\Delta R}$$

is kept substantially constant, the core being so designed as to compensate for changes in core loss with frequency.

Figure 9 is a cross section of a core with varying magnetic density. Portion 3 of said core is of comparatively low permeability and low losses at high frequencies. Portion 4 is an intermediate section of the core with medium permeability and losses. Portion 5 is a section of maximum permeability and higher losses at lower frequencies. These cores of varying magnetic density can be produced by subjecting separate sections to different pressures. A somewhat increased variation of magnetic density can be produced by an additional shaping of the core as shown in Figure 10, wherein the section 6 is of smaller diameter than the sections 7 and 8.

Another method of producing varying density is to press the cores in molds of such a shape that the pressure is not evenly distributed throughout the core. Figure 11 shows such a core, wherein the portions 9 and 10 of the center core, due to frictional losses on the wall of the mold, have lower magnetic density than the portions 11.

Still another method of producing varying density is to charge the mold with two or three different mixtures, in which the insulating coatings are of different thickness. Still another method to produce varying density is to use various sizes of magnetic material. A small particle size usually produces smaller permeability and smaller losses, coarser particles producing higher permeability with higher losses.

Cores made in quantity in the same mold in accordance with any of the above described methods will have substantially the same weights, dimensions and physical properties. However, small variations in the amount of magnetic and other materials may produce variations in magnetic and electrical properties of the cores. To obtain better uniformity, the completed cores may be tested and those having excess permeability may be reduced in size by any suitable mechanical method, so as to bring them into agreement with the standards.

In cores of movable type, it is quite essential to obtain uniformity of performance, especially when several cores are arranged to operate simultaneously and synchronously on several inductances. A very careful matching of effective permeabilities is required under these conditions. But, in spite of careful matching, the intermediate portions of the cores may not always produce the same inductance variations.

To compensate for this possible misalignment, an additional compensating pellet, such as shown in Figure 11, may be inserted in the main core. A small pellet 12 of magnetic material is placed in one end of the core 9, in a suitable cavity 13 provided to receive it. With the core inserted into the coil to a definite intermediate position, an adjustment of the effective permeability may be made either by altering the position of the pellet relatively to the core 9 or by selecting a proper size of pellet, and sealing it into the core. Experience shows that this adjustment produces no substantial change in the effective permeability of the complete core.

Other methods for intermediate adjustment are (1) to fill the cavity 13 with a sufficient quantity of loose insulated powdered material, and then seal the end; (2) to use a sufficient quantity of the insulated powder already mixed with the sealing compound; and (3) to use a solid core and bore a hole at the open end, thereby altering the effective air gap, until the core matches the standard.

When cores are pressed and taken out of the molds, the outer layer of particles has considerably less resistivity than the interior because of the friction of the mold walls and the consequent polishing effect on the outer surface. This decrease of resistivity sometimes is harmful at high frequencies, and continuity of the core-surface, therefore, may be broken by any suitable mechanical or chemical means such as sand blasting, pickling with acids, or parkerizing.

The shell-type cores shown in Figures 7, 8, 9 and 11 are especially advantageous in that they produce maximum permeability with minimum losses for a solenoidal coil. Coils of this type are recognized as most advantageous for high-frequency work because of their inherent low-loss properties. The shell 14, in this type of core, is united at one end with a central core 15 between which and said shell, is an annular cavity 16 for the reception of a solenoidal coil. The shell and the central core may be separately molded portions of the same material as shown in Figure 11, the two parts of the core unit being arranged to be held in proper magnetic and mechanical relation.

When in the claims I use the word "matured" or the word "mature", I have reference to oxidation or polymerization, either of which can be considered as a form of integration. Also, when I refer to the insulator as being "matured in situ", I mean that it is oxidized or polymerized after it is applied to the magnetic particles.

Having thus described my invention what I claim is:

1. A compressed comminuted magnetic material having individually-insulated particles and a substantially constant permeability for a band of radio frequencies at least one octave wide.

2. A compressed comminuted magnetic material having individually-insulated particles and a substantially constant permeability for a band of frequencies between 1 kilocycle and 500 kilocycles.

3. A compressed comminuted magnetic material having individually-insulated particles and a substantially constant permeability at frequencies of from 300 to 1400 kilocycles. 80
5. 4. A compressed comminuted magnetic material having individually-insulated particles and a substantially constant permeability for a range of magnetic intensities between .01 and 10 gauss. 85
10. 5. A compressed comminuted magnetic material having individually-insulated particles, and an apparent permeability of the order of 8 and a resistivity ranging from 10 to 50 ohms per centimeter cube. 90
15. 6. A compressed comminuted magnetic material having individually-insulated particles and an effective permeability of the order of 8, and a core loss of the order of .91 erg per cubic centimeter per cycle at unit induction and at a frequency of the order of 200 kilocycles. 95
20. 7. A compressed toroidal comminuted magnetic core having individually-insulated particles and a factor of merit of the order of  $3 \times 10^{-6}$  at a frequency of 500 kilocycles. 100
25. 8. A compressed cylindrical comminuted magnetic core having individually-insulated particles and a factor of merit of the order of  $25 \times 10^{-6}$  at a frequency of 500 kilocycles. 105
30. 9. A compressed comminuted magnetic core unit having individually-insulated particles and including a core and a shell of the same material adapted to receive between them a solenoidal coil, said core unit having an effective permeability of the order of 8 and a factor of merit of the order of  $10 \times 10^{-6}$  at a frequency of 500 kilocycles. 110
35. 10. A compressed comminuted magnetic core having magnetic density varying along its magnetic path, adapted to vary the inductance of a solenoidal coil while maintaining the ratio of inductance to resistance substantially constant. 115
40. 11. A compressed comminuted magnetic core containing varying quantities of magnetic material along its magnetic path, adapted to vary the inductance of a solenoidal coil while maintaining the ratio of inductance to resistance substantially constant. 120
45. 12. A compressed comminuted magnetic core for an inductance coil, said core having gradually varying magnetic density along its magnetic path. 125
50. 13. A compressed comminuted magnetic core for an inductance coil, said core having varying degrees of magnetic density along its magnetic path and so arranged that the lower degree of magnetic density is adjacent to the air gap included in said path. 130
55. 14. A compressed comminuted magnetic core having magnetic density varying along its magnetic path in such a manner as to compensate for changes in core losses with frequency, to thereby maintain the factor of merit substantially constant. 135
60. 15. A compressed comminuted magnetic core having insulated particles and having an apparent permeability of not less than 7 and a resistivity of at least 10 ohms per centimeter cube, and having an internal portion adapted to adjustably occupy the space within a coil, and an external portion adapted to adjustably occupy the space immediately surrounding said coil, and forming a magnetic circuit containing an air gap. 140
65. 16. A compressed comminuted magnetic core having insulated particles and having an apparent permeability of not less than 7 and a resistivity of at least 10 ohms per centimeter cube, 145
70. and having an internal portion adapted to adjustably occupy the space within a solenoidal coil, and an external portion adapted to adjustably occupy the space immediately surrounding said coil, said two portions being united at one end, and forming a magnetic circuit containing an air gap. 80
75. 17. A compressed comminuted magnetic core having insulated particles and having an internal portion adapted to adjustably occupy the space within a solenoidal coil, and an external portion adapted to adjustably occupy the space immediately surrounding said coil, said two portions being united at one end, said magnetic core having varying magnetic density along its magnetic path. 85
18. A compressed comminuted magnetic core comprising a central portion and a shell portion surrounding the central portion and forming an annular gap between said two portions, which gap is adapted to receive a solenoidal coil, said core having sections of varying magnetic density along its magnetic path. 90
19. A compressed comminuted magnetic core having a tapered portion and having different degrees of magnetic density along its magnetic path. 95
20. A compressed magnetic core carrying at one end a standardizing magnetic mass. 100
21. A compressed magnetic core having at one end a cavity for the reception of a standardizing magnetic mass. 105
22. The process of standardizing a compressed comminuted magnetic core, which consists in varying the cross-section of the magnetic circuit of said core at a desired portion. 110
23. The process of standardizing a compressed comminuted magnetic core, which consists in varying the cross-section of the magnetic circuit of said core, at a point adjacent to an air gap. 115
24. The process of standardizing a compressed comminuted magnetic core, which consists in varying the cross-section of the magnetic circuit of said core, at a point adjacent to an air gap, where such variation produces least effect on the effective permeability of the complete core. 120
25. A compressed comminuted magnetic core having individually-insulated particles and a broken outside surface which increases the resistivity of the surface layer. 125
26. A powdered magnetic material of low coercivity, consisting of particles approximating in size .005 millimeter, the particles being substantially insulated by thin films of insoluble heat-resisting material. 130
27. A powdered magnetic material consisting of particles approximating in size .005 millimeter, the particles being substantially insulated by thin films of chemically-stable and pressure-resisting material of organic nature. 135
28. A powdered magnetic material, the particles whereof are approximately .005 millimeter in size and are substantially insulated by an organic material matured in situ. 140
29. A powdered magnetic material, the particles whereof are small enough to pass through a screen of 400 meshes per inch and are substantially insulated by an organic material matured in situ by heat treatment. 145
30. A powdered magnetic material, the particles whereof are substantially insulated by an oxidized varnish. 150
31. A powdered magnetic material, the particles whereof are substantially insulated by an oxidized

varnish which is of the order of 3% of the weight of the magnetic material.

32. A powdered magnetic material, the particles whereof are substantially insulated by an oxidized China-wood oil varnish.

33. The process of insulating powdered magnetic material, which consists in coating the particles of said material with a fluent organic substance, and maturing the coatings by heat treatment while maintaining the material in the powdered form.

34. The process of insulating powdered magnetic material, which consists in coating the particles of said material with a fluent oxidizing organic substance, and maturing the coatings by heat treatment while maintaining the material in the powdered form.

35. The process of insulating powdered magnetic material, which consists in coating the particles of said material with a fluent China-wood oil varnish, and maturing the coatings by heat treatment while maintaining the material in the powdered form.

36. The process of insulating powdered magnetic material, which consists in coating the particles of said material with films of a quick-oxidizing fluent substance, and completing the oxidation of said films by heat treatment, while maintaining the material in the powdered form.

37. The process of making a comminuted magnetic core, which consists in coating magnetic particles with organic insulating films, mixing the coated particles with a binding material, softening said binding material to render it plastic, and subjecting the entire mass to pressure in a mold while said binder is still plastic.

38. The process of producing a comminuted magnetic core, which consists in coating magnetic particles with organic insulating films, mixing a binder with the insulated particles to produce a coherent mass, placing said coherent mass in a mold, rendering said mass plastic, and then subjecting said mass to a pressure of from 5 to 25 tons per square inch, depending upon the shape of the core, to thereby reduce it to the desired volume.

39. The process of producing a comminuted magnetic core, which consists in coating magnetic particles with elastic insulating films, mixing a phenolic resin binder with the insulated particles to produce a coherent mass, placing said coherent mass in a mold, subjecting said mass, while at a temperature approximating 100° C., to a pressure of from 5 to 25 tons per square inch, depending upon the shape of the core, to thereby reduce it to the desired volume, and then baking the compressed core to thereby convert the phenolic resin binder into a chemically-stable bakelite.

40. A magnetic material including magnetic particles, China-wood oil varnish and a phenolic resin, said China-wood oil varnish being in quantity not more than 3% of the weight of the material, and said phenolic resin being in quantity not more than 7% of the weight of said material.

41. The process of insulating powdered magnetic material, which consists in coating the particles of said material with an organic substance, and then integrating the substance of said coatings while maintaining the material in the powdered form.

42. The process of insulating powdered magnetic material, which consists in coating the particles of said material with a fluent organic substance, and then treating the coatings of said substance to render them insoluble, while maintaining the material in the powdered form.

43. The process of producing insulated magnetic particles, which consists in coating said particles with an organic substance, and subjecting said coated particles to heat treatment until the organic substance is so matured as to constitute insulating elastic films on said particles.

44. The process of making a core of comminuted magnetic material, which consists in coating the particles of said material with an elastic insulating substance, mixing said insulated particles with a binder, compressing the mixture in a mold, removing the molded compressed core and treating said core to release the compression of said elastic substance while the binder is in a softened state.

45. The process of producing a magnetic core of comminuted magnetic material, which consists in coating the particles of said material with an organic insulating substance dissolved in a solvent, evaporating said solvent while agitating the particles, mixing said particles after the coating is dry with a binder, and subjecting said mixture to heat and pressure in a mold at a temperature sufficient to soften said binder.

46. The process of producing a magnetic core of comminuted magnetic material, which consists in coating the particles of said material with a fluent insulating substance containing volatile matter, evaporating the volatile matter while the particles are being coated and agitated, and continuing the agitation until the particles are coated with a dry elastic film, mixing a binder with said insulated particles, subjecting the mixture to heat and pressure in a mold at a temperature sufficient to soften the binder, removing the core from the mold and subjecting the core to treatment which slightly increases its dimensions and materially reduces its electrical losses.

47. The process of making a core of comminuted magnetic material, which consists in insulating the individual particles of said magnetic material, mixing the insulated particles with an unmatured binder, binding said insulated particles together under pressure, and then releasing the pressure and completing the maturing of said unmatured product.

48. The process of making a core of comminuted magnetic material, which consists in insulating the individual particles of said magnetic material, mixing said insulated particles with a binder, binding said insulated particles together under pressure in a mold to produce the core, removing said core from the mold in order to release the pressure, and heat treating said core to slightly increase its dimensions and to materially reduce its electrical losses.

49. The process of decreasing the electrical losses of a compressed material made from finely-divided insulated magnetic particles, which consists in treating the material to secure a permanent increase in its physical dimensions.

50. Powdered iron, chemically reduced as by hydrogen, the greater portion of the particles thereof being small enough to pass through a screen of 400 meshes to the inch and being substantially insulated by an oxidized varnish.

51. Powdered iron, chemically reduced as by hydrogen, the particles thereof being small enough to pass through a screen of 400 meshes to the inch and being insulated by an oxidized China-wood oil varnish.

52. Powdered iron, chemically reduced as by hydrogen, the particles thereof being small

- enough to pass through a screen of 400 meshes to the inch and being substantially insulated by an organic material matured in situ. 80
53. Powdered iron, chemically reduced as by hydrogen, the particles thereof being small enough to pass through a screen of 400 meshes to the inch and being substantially insulated by a chemically-stable and pressure-resisting material of organic nature. 85
54. Powdered iron, chemically reduced as by hydrogen, the particles whereof are substantially insulated by an elastic substance which is of the order of 3% of the weight of the powdered iron. 90
55. Powdered iron, chemically reduced as by hydrogen, consisting of particles approximating in size .005 millimeter, the particles being substantially insulated by thin films of insoluble, elastic material. 95
56. Powdered iron, chemically reduced as by hydrogen, consisting of particles approximating in size .005 millimeter, the particles being substantially insulated by thin films of organic material chemically changed in situ. 100
57. A powdered magnetic material of low coercivity, consisting of particles approximating in size .005 millimeter, the particles being substantially insulated by thin films of heat-resisting material. 105
58. A magnetic material including magnetic particles small enough to pass through a screen of 400 meshes to the inch, and a chemically-converted insulating organic substance in quantity of the order of 3% of the weight of the material. 110
59. Compressed magnetic material including individually-insulated magnetic particles of such dimensions and so closely related that said material has a factor of merit ranging from  $3 \times 10^{-6}$  to  $25 \times 10^{-6}$  at a frequency of 500 kilocycles in cores of various shapes. 115
60. Compressed magnetic material including individually-insulated magnetic particles of such dimensions and so closely related that said material has an apparent permeability of the order of 8, and a factor of merit ranging from  $3 \times 10^{-6}$  to  $25 \times 10^{-6}$  at a frequency of 500 kilocycles in cores of various shapes. 120
61. Compressed magnetic material including individually-insulated magnetic particles of such dimensions that the majority of the particles will pass through a screen having 400 meshes to the inch and so closely related that said material has a factor of merit ranging from  $3 \times 10^{-6}$  to  $25 \times 10^{-6}$  at a frequency of 500 kilocycles in cores of various shapes. 125
62. Compressed magnetic material including individually-insulated magnetic particles of such dimensions that the majority of the particles will pass through a screen having 400 meshes to the inch and so closely related that said material has an apparent permeability of the order of 8, and a factor of merit ranging from  $3 \times 10^{-6}$  to  $25 \times 10^{-6}$  at a frequency of 500 kilocycles in cores of various shapes. 130
63. The process of producing a magnetic core of comminuted magnetic material, which consists in coating the particles of said material with an organic insulating substance dissolved in a solvent, evaporating said solvent while agitating the particles, heat treating the insulated particles, mixing said particles with a binder after the coating is dry and subjecting said mixture to heat and pressure in a mold at a temperature sufficient to soften said binder. 140
64. The process of insulating powdered magnetic material, which consists in coating the particles of said material with a fluent organic substance and then treating said coatings to mature the same while maintaining the material in the powdered form. 145
65. A compressed comminuted magnetic core unit having individually-insulated particles and including a core and a shell of the same material adapted to receive between them a solenoidal coil, said core unit having a factor of merit of the order of  $10 \times 10^{-6}$  at a frequency of 500 kilocycles. 150
66. The process of improving the electrical characteristics of a compressed comminuted magnetic core including a binder, and particles insulated by an elastic substance, which consists in rendering the binder plastic and releasing the compression so as to produce an increase in the physical dimensions of the core before the binder is solidified. 155
67. The process of decreasing the electrical losses of a compressed comminuted magnetic body including bonded particles insulated by an elastic substance, which consists in maintaining the binder in a plastic condition and releasing the compression so as to produce an increase in the physical dimensions of the body before the binder is matured. 160
68. The process of decreasing the electric losses of a compressed comminuted magnetic core including bonded particles insulated by an elastic substance, which consists in rendering the binder plastic and releasing the compression so as to produce an increase in the physical dimensions of the core before the binder is matured. 165
69. The process of improving the electrical characteristics of a compressed comminuted magnetic body including bonded particles insulated by an elastic substance, which consists in rendering the binder plastic and releasing the compression so as to produce increased separation of the magnetic particles before the binder is solidified. 170
70. The process of completing a moulded and compressed magnetic core having an elastic substance between the particles of said core, which consists in releasing the pressure in said core to thereby permit said elastic substance to separate contacting particles of said core. 175
71. The process of making a magnetic material, which consists in coating magnetic particles with organic insulating films, mixing the coated particles with a binding substance, softening said binding substance to render it plastic, and subjecting the mixture to pressure while the binder is still plastic. 180
72. The process of decreasing the electrical losses of a compressed comminuted magnetic core including a binder, which consists in rendering the binder plastic and thereby releasing the compression so as to produce an increase in the physical dimensions of the core before the binder is solidified. 185
73. The process of producing a comminuted magnetic core, which consists in coating magnetic particles with insulating films, mixing a binder with the insulated particles, placing said mixture in a mold, subjecting said mixture while the binder is in a plastic condition to a pressure of from 5 to 25 tons per square inch, depending upon the shape of the core, to thereby reduce it to the desired volume, and then treating the core outside of the mold to permit it to expand so as to reduce its electrical losses. 190
74. Compressed magnetic material including minute magnetic particles, characterized in that substantially all of said magnetic particles are 195

capable of passing through a 400-mesh screen and are insulated, and that the compressed material has an apparent permeability of not less than 7 and a resistivity of at least 10 ohms per centimeter cube.

75. Compressed magnetic material including insulated magnetic particles of such dimensions and so closely related that said compressed material has an apparent permeability of not less than 7 and a resistivity of at least 10 ohms per centimeter cube.

76. Compressed magnetic material including magnetic particles approximating in size .005 millimeter, said particles being insulated and so closely related that said compressed material has an apparent permeability of not less than 7 and a resistivity of at least 10 ohms per centimeter cube.

77. A compressed comminuted magnetic core containing magnetic particles fine enough to pass through a screen having 400 meshes to the inch, said core having an effective permeability of not less than 4 and a resistivity of at least 10 ohms per centimeter cube.

78. The process of producing a comminuted magnetic core, which consists in individually insulating finely divided magnetic particles with organic films, mixing said insulated particles with a powdered binder, placing said mixture in a mould, subjecting said mixture to pressure while the binder is in a plastic condition to thereby reduce said mixture to the desired volume, and then heat treating the core to reduce its eddy current losses.

79. The process of producing a comminuted magnetic core from magnetic particles individually insulated with an organic coating, which consists in mixing said insulated particles with a powdered binder, placing said mixture in a mould, heating the mould to render the binder plastic, subjecting said mixture to pressure, removing the compressed core body from the mould and heat treating said compressed body to reduce its eddy current losses.

WLADIMIR J. POLYDOROFF.

28

CERTIFICATE OF CORRECTION.

Patent No. 1,982,689.

December 4, 1934

WLADIMIR J. POLYDOROFF.

It is hereby certified that error appears in the printed specification of the above numbered patent requiring correction as follows: Page 3, first column, line 10, for "passing" read pressing; and that the said Letters Patent should be read with this correction therein that the same may conform to the record of the case in the Patent Office.

Signed and sealed this 31st day of March, A. D. 1936.

(Seal)

50

Leslie Frazer  
Acting Commissioner of Patents.

125

15

130

80

185

5

140

85

145

5

150

capable of passing through a 400-mesh screen and are insulated, and that the compressed material has an apparent permeability of not less than 7 and a resistivity of at least 10 ohms per centimeter cube.

75. Compressed magnetic material including insulated magnetic particles of such dimensions and so closely related that said compressed material has an apparent permeability of not less than 7 and a resistivity of at least 10 ohms per centimeter cube.

76. Compressed magnetic material including magnetic particles approximating in size .005 millimeter, said particles being insulated and so closely related that said compressed material has an apparent permeability of not less than 7 and a resistivity of at least 10 ohms per centimeter cube.

77. A compressed comminuted magnetic core containing magnetic particles fine enough to pass through a screen having 400 meshes to the inch, said core having an effective permeability of not less than 4 and a resistivity of at least 10 ohms per centimeter cube.

78. The process of producing a comminuted magnetic core, which consists in individually insulating finely divided magnetic particles with organic films, mixing said insulated particles with a powdered binder, placing said mixture in a mould, subjecting said mixture to pressure while the binder is in a plastic condition to thereby reduce said mixture to the desired volume, and then heat treating the core to reduce its eddy current losses.

79. The process of producing a comminuted magnetic core from magnetic particles individually insulated with an organic coating, which consists in mixing said insulated particles with a powdered binder, placing said mixture in a mould, heating the mould to render the binder plastic, subjecting said mixture to pressure, removing the compressed core body from the mould and heat treating said compressed body to reduce its eddy current losses.

WLADIMIR J. POLYDOROFF.

28

CERTIFICATE OF CORRECTION.

Patent No. 1,982,689.

December 4, 1934

WLADIMIR J. POLYDOROFF.

It is hereby certified that error appears in the printed specification of the above numbered patent requiring correction as follows: Page 3, first column, line 10, for "passing" read pressing; and that the said Letters Patent should be read with this correction therein that the same may conform to the record of the case in the Patent Office.

Signed and sealed this 31st day of March, A. D. 1936.

(Seal)

50

Leslie Frazer  
Acting Commissioner of Patents.

125

15

130

80

185

5

140

85

145

5

150